

## UNITED STATES PATENT OFFICE

2,064,031

## CONCENTRATION OF MINERALS

Oliver C. Ralston, Clarkdale, Ariz., assignor, by  
mesne assignments, to Phelps Dodge Corpora-  
tion, New York, N. Y., a corporation of New  
York

No Drawing. Application October 6, 1930,  
Serial No. 486,746

## 10 Claims. (Cl. 209—167)

This invention relates to the concentration of minerals and has for an object the provision of an improved process for concentrating minerals by froth flotation. More particularly, the invention contemplates the provision of an improved method for controlling the extraction of valuable minerals and grade of concentrate produced.

In froth flotation processes, it is customary to conduct one flotation operation for the purpose of obtaining a rougher concentrate and then subject the rougher concentrate to a second flotation operation for the purpose of obtaining a concentrate containing a higher percentage of the valuable mineral, the tailings from the second operation being mixed with the feed treated during the first operation.

The tailings from the first or rougher operation may be wasted, so it is important that the operation be so conducted that maximum extraction be accomplished. Since the rougher concentrates are retreated, grade of concentrate may be sacrificed in favor of extraction in the rougher operation. The tailings from the second or cleaner operation are retreated in the rougher operation, so extraction may be sacrificed in favor of grade of concentrate in the cleaner operation.

I have discovered that improved results may be obtained by controlling the densities of the pulps employed in the rougher and cleaner operations. I have found that grade of concentrate obtained improves and extraction becomes poorer as pulp density increases. I, therefore, propose to employ a pulp of relatively low density in conducting the rougher operation and a pulp of relatively high density in conducting the cleaner operation. I have discovered that improved extractions and improved grades of concentrates are obtained when pulps containing not more than about forty percent solids, by weight, are employed in the rougher operations and when pulps of greater densities than the pulps employed in the rougher operations are employed in the cleaner operations. I have also discovered that improved grades of concentrates may be obtained by regrounding the rougher concentrates before subjecting them to the cleaner operation.

The relative pulp densities employed in the rougher and cleaner operations in the treatment of any particular ore will be determined by the natures of the minerals in the ore. In treating ores containing minerals having relatively low specific gravities, pulps containing relative-

ly low percentages of solids, by weight, may be employed.

The following table illustrates the results obtained in treating reground rougher zinc concentrates obtained by treating United Verde mine ore in which zinc is present in the form of marmatite:—

| Cleaner feed<br>percent solids | Concentrates<br>percent Zn | Extraction<br>(percent) |    |
|--------------------------------|----------------------------|-------------------------|----|
| 10                             | 31.5                       | 76.5                    | 10 |
| 20                             | 27.5                       | 82.5                    |    |
| 30                             | 27.0                       | 85.5                    |    |
| 40                             | 29.5                       | 85.5                    |    |
| 45                             | 31.5                       | 84.8                    |    |
| 50                             | 32.5                       | 83.5                    | 15 |
| 55                             | 33.5                       | 82.5                    |    |

The above results were obtained by varying the pulp density and maintaining other conditions constant. The cleaner circuit was operating on a reground rougher concentrate assay-ing about 16% Zn. The cleaner tailings were returned continuously to the head of the rougher circuit.

The results obtained show that cleaner operations employing pulps containing about ten percent or less of solids produce concentrates corresponding in grade to those produced when pulps containing about forty-five percent solids are employed. The extraction, however, is better when the higher density pulps are used, and I, therefore, prefer to employ such pulps in cleaner operations.

A complete process of the invention for treat-ing an ore of the type of United Verde mine ore involves grinding of the ore to a suitable par-ticle size, treatment of the ground product in a pulp containing not more than about forty per-cent solids with the addition of suitable flo-tation agents to produce a rougher concentrate, thickening of the rougher concentrate to obtain a pulp containing not less than about forty per-cent solids, treatment of the thickened pulp with the addition of suitable flotation agents to produce a cleaner concentrate and a cleaner tailing, and return of the cleaner tailing to the rougher circuit.

The rougher concentrate may be reground be-fore being subjected to the cleaner operation. Regrinding is preferably conducted after the rougher concentrate pulp has been thickened. Thickening or dewatering of the rougher con-centrate may be conducted in any suitable man-ner.

I claim:—

1. The method of concentrating minerals which comprises subjecting the mineral in a relatively low-density pulp to a froth flotation operation to produce a rougher concentrate, the density of the pulp employed in the production of the rougher concentrate being such as to provide for optimum recovery of valuable mineral, and subjecting the rougher concentrate to a froth 5 flotation operation in a relatively higher density pulp, the density of the pulp employed in treating the rougher concentrate being such as to provide for the production of a concentrate of optimum quality.
- 10 2. The method of concentrating minerals, which comprises subjecting the mineral in the form of a relatively low density pulp to a froth flotation operation to produce a rougher concentrate, forming a high density pulp of the rougher concentrate, and subjecting the resulting pulp to a second froth flotation operation, the pulp treated in said second froth flotation operation being of a substantially higher density than the pulp employed in forming the rougher concentrate.
- 15 3. The method of concentrating minerals, which comprises subjecting the mineral to a froth flotation operation in a relatively low density pulp to produce a rougher concentrate, 20 grinding the rougher concentrate, forming a pulp of the rougher concentrate of substantially higher density than that employed in obtaining the rougher concentrate, and subjecting the resulting pulp to a second froth flotation operation.
- 25 4. The method of treating sulphide ores, which comprises subjecting the ore in the form of a pulp to a froth flotation operation to produce a rougher concentrate, forming a pulp of the rougher concentrate of substantially higher 30 density than that employed in obtaining the rougher concentrate and containing not less than about forty percent solids, and subjecting the resulting pulp to a second froth flotation operation.
- 35 5. The method of treating sulphide ores, which comprises subjecting the ore in the form of a pulp to a froth flotation operation to obtain a rougher concentrate, grinding the rougher concentrate, forming a pulp of the rougher 40 concentrate of substantially higher density than that employed in obtaining the rougher concentrate and containing not less than about forty percent solids, and subjecting the resulting pulp to a second froth flotation operation.
- 45 6. The method of treating sulphide ores, 50 which comprises subjecting the ore in the form of a low density pulp containing not more than about forty percent solids to a froth flotation operation to produce a rougher concentrate, forming a high density pulp of the rougher concentrate, and subjecting the resulting pulp to a second froth flotation operation, the pulp treated in said second froth flotation operation being of a substantially higher density than the pulp employed in forming the rougher concentrate.
- 55 7. The method of treating sulphide ores, which comprises subjecting the ore in the form of a low density pulp containing not more than about forty percent solids to a froth flotation operation to produce a rougher concentrate, grinding the rougher concentrate, forming a high density pulp of the rougher concentrate, and subjecting the resulting pulp to a second froth flotation operation, the pulp treated in said second froth flotation operation being of a substantially higher density than the pulp employed in forming the rougher concentrate.
- 60 8. The method of treating sulphide ores, which comprises subjecting the ore in the form of a low density pulp containing not more than about forty percent solids to a froth flotation operation to produce a rougher concentrate, dewatering the rougher concentrate to produce a pulp of substantially higher density than that employed in obtaining the rougher concentrate, subjecting the concentrate in the higher density pulp to a grinding operation, and subjecting the resulting pulp to a froth flotation operation.
- 65 9. The method of treating sulphide ores, which comprises subjecting the ore in the form of a low density pulp containing not more than about forty percent solids to a froth flotation operation to produce a rougher concentrate, subjecting the rougher concentrate to a wet grinding operation, dewatering the resulting pulp to produce a pulp of substantially higher density than that employed in obtaining the rougher concentrate, and subjecting the higher density pulp to a froth flotation operation.
- 70 10. The method of treating sulphide ores, which comprises subjecting the ore in the form of a low density pulp containing not more than about forty percent solids to a froth flotation operation to produce a rougher concentrate, forming a high density pulp of the rougher concentrate, and subjecting the resulting pulp to a second froth flotation operation, the pulp treated in said second froth flotation operation being of a substantially higher density than the pulp employed in forming the rougher concentrate.

OLIVER C. RALSTON.